

## UNITED STATES PATENT OFFICE

ARMAN E. BECKER, OF NEWARK, NEW JERSEY, ASSIGNOR TO STANDARD OIL DEVELOPMENT COMPANY, A CORPORATION OF DELAWARE

## LUBRICANT

No Drawing.

Application filed November 28, 1923. Serial No. 677,512.

This invention relates to lubricants and their preparation, and will be fully understood from the following description.

In the cracking of hydrocarbon oils by pressure distillation, etc., the residuum remaining is a tarry-appearing liquid customarily regarded as usable only for fuels. I have found however that from such material there can be prepared lubricants suitable for certain uses. To segregate the best portions I subject such residuum to distillation, preferably under a vacuum or by use of steam, and take off the lighter fractions separately and then the heavier, down to a pitch bottom.

Depending upon the particular stock which has been used as starting material, more or less of the fractions can be saved after the very lightest. By distilling on ten percent cuts, all fractions that have any utility either alone or for blending can be conveniently separated and handled. In some cases so much paraffine wax is present in the distillates, that it is worth while to chill and press in order to secure an oil with a better cold test.

Having obtained the desired cuts, I then proceed to work them up in accordance with the particular products wanted. Some of the cuts can be used as they are. In other instances I blend down heavier cuts with selected lighter cuts or blend variously with ordinary lubricating oils. In some cases I further improve the quality by an acid treatment for instance 10-30 lbs. of 66° Bé. sulfuric acid to the barrel of oil. In other cases for special uses I add sulfur, 1-5% for example, to selected fractions and heat to around 400-500° F. until the sulfur dissolves. This product can be used as such or can be blended down with other fractions or with ordinary lubricating oils.

As illustrating the invention, but without at the same time implying any limitations, the following examples may be noted:

I. A residuum (of residual oil 23.9° Bé. gravity) from pressure distillation cracking Mid-Continent gas oil was distilled under a vacuum, by 10% cuts. The heavier cuts showed the following properties:

| Cut    | Gravity            | Saybolt viscosity @ 100° F. | Saybolt viscosity @ 212° F. | Flash | 50 |
|--------|--------------------|-----------------------------|-----------------------------|-------|----|
| 60-70% | 26.7° Bé.          | 55                          |                             | 330   |    |
| 70-80  | 25.1               | 68                          |                             | 330   | 55 |
| 80-90  | 17.1               | 160                         | 42                          | 330   |    |
| 90-97  | Heavier than water | 1895                        | 91                          | 335   |    |

A portion of cut 80-90 (flash 360) was then combined with sulfur by adding 2% of sulfur and heating to 400-450° F.; and another portion was also combined with sulfur by adding 5% of sulfur and heating in similar manner. Also a portion of cut 90-97 (flash 365) was combined with sulfur by adding 2% of sulfur and another portion was combined with sulfur by adding 5% of sulfur and heating. The products showed the following properties:

| Cut                     | Gravity            | Saybolt viscosity @ 100° F. | Saybolt viscosity @ 212° F. | 70 |
|-------------------------|--------------------|-----------------------------|-----------------------------|----|
| 80-90 (2% sulfur added) | 16.2° Bé.          | 208                         | 42                          |    |
| 80-90 (5% sulfur added) | 14.1               | 194                         | 44                          |    |
| 90-97 (2% sulfur added) | Heavier than water |                             | 133                         | 75 |
| 90-97 (5% sulfur added) | do                 |                             | 103                         |    |

20 parts of cut 60-70 were blended with 80 parts of an ordinary spindle lubricating oil (of 31° Bé. gravity, and Saybolt viscosity 103 at 100° F.). The product showed the following properties:

| Gravity   | Saybolt viscosity @ 100° F. | 85 |
|-----------|-----------------------------|----|
| 30.8° Bé. | 89                          |    |

30 parts of cuts 80-97 (with flash 360), to which had been added 5% of sulfur with 90

heating to 400-425° F., was blended with 70 parts of the straight cuts 60-80 (of flash between 280 and 360). The product showed the following properties:

| 5  | Gravity       | Saybolt viscosity @ 100° F. | Saybolt viscosity @ 212° F. | Flash |
|----|---------------|-----------------------------|-----------------------------|-------|
| 10 | 21.3° Bé..... | 81                          | 37                          | 310   |

15 30 parts of cuts 80-97 to which had been added 5 parts of sulfur with heating was blended with 70 parts of an ordinary spindle lubricating oil (of 31° Bé. gravity, and Saybolt viscosity 103 at 100° F.). This product showed the following properties:

| 20            | Gravity | Saybolt viscosity @ 100° F. | Saybolt viscosity @ 212° F. | Flash |
|---------------|---------|-----------------------------|-----------------------------|-------|
| 24.6° Bé..... |         | 151                         | 43                          | 350   |

25 II. A residuum (of 22.4° Bé. gravity) from pressure cracking Mid-Continent gas oil was distilled until 70% was driven off. The bottoms showed a gravity heavier than water, and a Saybolt viscosity of 96 at 212° F.

30 A portion of the bottoms was combined with sulfur by adding 2% of sulfur and heating to 400-450° F., and another portion was similarly combined with sulfur by adding 5% of sulfur and heating. These products showed the following properties:

| 35                             | Gravity                 | Saybolt viscosity @ 212° F. |
|--------------------------------|-------------------------|-----------------------------|
| Bottoms (2% sulfur added)..... | Heavier than water..... | 143                         |
| Bottoms (5% sulfur added)..... | do.....                 | 159                         |

40 45 30 parts of the bottoms with the 5% sulfur was blended with 70 parts of the straight 60-70 cuts. The product showed the following properties:

| 50            | Gravity | Saybolt viscosity @ 100° F. | Saybolt viscosity @ 212° F. |
|---------------|---------|-----------------------------|-----------------------------|
| 19.8° Bé..... |         | 160                         | 44                          |

55 30 parts of the bottoms with the 5% sulfur was blended with 70 parts of an ordinary spindle lubricating oil (of 31° Bé. gravity, and Saybolt viscosity 103 at 100° F.). This product showed the following properties:

| 60            | Gravity | Saybolt viscosity @ 212° F. |
|---------------|---------|-----------------------------|
| 23.7° Bé..... |         | 51                          |

65 As seen, products derived in accordance with this invention are characterized by a relatively low viscosity for any given Baumé

gravity as compared with ordinary lubricating oils of the same gravity; and where sulfur has been added the sulfur content is at least 0.35%.

A typical lubricating composition prepared according to my invention comprises a residual oil having a gravity of 21-22° Bé., a Saybolt viscosity of 78-85 at 100° F., a flash of 300-315, and containing at least 0.5% of combined sulfur. Another typical composition which may be mentioned by way of illustration contains a residual oil having a gravity between 25 and 31° Bé., a Saybolt viscosity between 150 and 90 at 100° F., and contains at least 0.5% of combined sulfur.

What I claim is:

1. A process of preparing lubricants, which comprises distilling a residuum from cracking of petroleum, segregating cuts of the distillate and blending with another oil.

2. A lubricant comprising hydrocarbon oil constituents from residuum of cracking petroleum, and containing at least 0.35% of combined sulfur and not substantially more than 5% of such sulfur.

3. The method of making a lubricating oil from pressure distillation cracking residuum which comprises distilling such a residuum to segregate distillates therefrom having lubricating characteristics, adding sulphur to a distillate so segregated and heating until the sulphur dissolves.

4. Method according to claim 3, in which the distillation, to segregate distillates, is conducted under vacuum.

5. Method according to claim 3, in which the oil with the added sulphur is heated to a temperature of between substantially 400° and 500° F. for a period sufficient to completely dissolve the sulphur.

6. Method, according to claim 3, in which the added sulphur is in amount not exceeding 5% of the oil to which it is added.

7. Method of making lubricating oil from pressure distillation cracking residuum which comprises distilling such a residuum to segregate a distillate therefrom having a viscosity in excess of 80 seconds Saybolt at 100° F., adding to such distillate sulphur and heating until the sulphur dissolves.

8. Method according to claim 7, in which the oil is heated to a temperature of between 400° and 500° F. until the sulphur dissolves.

ARMAN E. BECKER.

125

126